



US007673497B2

(12) **United States Patent**  
**Quest et al.**

(10) **Patent No.:** **US 7,673,497 B2**  
(45) **Date of Patent:** **\*Mar. 9, 2010**

(54) **SYSTEM, METHODS, AND COMPOSITIONS  
FOR DETECTING AND INHIBITING LEAKS  
IN TRANSMISSION SYSTEMS**

(75) Inventors: **William J. Quest**, Dallas, TX (US);  
**Darrell W. Patton**, Andover, KS (US)

(73) Assignee: **IDQ Operating, Inc.**, Garland, TX (US)

(\*) Notice: Subject to any disclaimer, the term of this patent is extended or adjusted under 35 U.S.C. 154(b) by 642 days.

This patent is subject to a terminal disclaimer.

(21) Appl. No.: **11/253,068**

(22) Filed: **Oct. 18, 2005**

(65) **Prior Publication Data**

US 2007/0087945 A1 Apr. 19, 2007

(51) **Int. Cl.**

*G01M 3/04* (2006.01)  
*C10M 137/10* (2006.01)  
*C09K 3/10* (2006.01)  
*C09K 11/06* (2006.01)  
*G01N 21/00* (2006.01)

(52) **U.S. Cl.** ..... **73/40.7**; 508/433; 508/579; 508/485; 508/591; 508/482; 106/33; 422/55; 422/61; 422/71; 252/68; 252/71; 252/72; 252/73; 252/77; 252/79; 252/301.16

(58) **Field of Classification Search** ..... 508/433, 508/579, 485, 591, 482; 106/33; 252/68, 252/72, 73, 77, 71, 79, 301.16; 73/40.7; 422/55, 61, 71

See application file for complete search history.

(56) **References Cited**

U.S. PATENT DOCUMENTS

4,662,940 A 5/1987 Monier  
4,664,825 A \* 5/1987 Walsh ..... 508/331

5,149,453 A \* 9/1992 Parekh ..... 252/68  
5,918,269 A 6/1999 Mahaffey, Jr.  
5,979,226 A 11/1999 Cavestri et al.  
6,070,454 A 6/2000 Cavestri  
6,070,455 A 6/2000 Cavestri  
6,101,867 A 8/2000 Cavestri  
6,150,306 A 11/2000 Friswell  
6,165,384 A 12/2000 Cooper et al.  
6,170,320 B1 1/2001 Scaringe et al.  
6,786,960 B2 9/2004 Profetto  
6,840,990 B2 1/2005 Gallagher et al.  
2005/0019236 A1 \* 1/2005 Martin et al. ..... 422/255  
2005/0269840 A1 \* 12/2005 Finerman et al. ..... 296/210

FOREIGN PATENT DOCUMENTS

WO WO 92/07249 4/1992

OTHER PUBLICATIONS

Co-pending U.S. Appl. No. 11/253,078 entitled "Systems, Methods, and Compositions for Detecting and Inhibiting Leaks in Engine Oil Systems," to Quest et al., filed Oct. 18, 2005; available in the private Patent Application Information Retrieval database.

Co-pending U.S. Appl. No. 11/253,076 entitled "Systems, Methods, and Compositions for Detecting and Inhibiting Leaks in Steering Systems," to Quest et al., filed Oct. 18, 2005; available in the private Patent Application Information Retrieval database.

\* cited by examiner

*Primary Examiner*—Glenn A Calderola

*Assistant Examiner*—Vishal Vasisth

(74) *Attorney, Agent, or Firm*—Meyertons, Hood, Kivlin, Kowert & Goetzel, P.C.; Eric B. Meyertons

(57) **ABSTRACT**

System, methods, and compositions are described for detecting and inhibiting leaks of a transmission system. The composition may include one or more transmission system sealants and one or more light activated compounds. The transmission system sealant(s) inhibit one or more of the leaks in the transmission system. One or more of the light activated compounds are visible when activating light is directed towards a portion of the exterior of the transmission system.

**13 Claims, No Drawings**

## SYSTEM, METHODS, AND COMPOSITIONS FOR DETECTING AND INHIBITING LEAKS IN TRANSMISSION SYSTEMS

### BACKGROUND

#### 1. Field of the Invention

The present invention relates generally to sealing and detecting leaks. More particularly, the invention relates to systems, methods, and compositions for sealing and detecting leaks in a transmission system.

#### 2. Description of the Relevant Art

Leak detection methods have been developed to analyze fluid systems, such as climate control systems, hydraulic systems, engine oil systems, power transmission systems, fuel systems, brake systems, or radiator coolant systems using dyes that fluoresce or phosphoresce. These dyes may be added to the system, circulated through the system, and then visualized using a light source. Once the origin of the leak is determined, the leak may be repaired mechanically or a sealant may be added to the system to stop the leak.

Sealant compositions and dyes are described in U.S. Pat. No. 4,662,940 to Monier; U.S. Pat. No. 5,918,269 to Mchaffey, Jr.; U.S. Pat. No. 5,979,226 to Cavestri; U.S. Pat. No. 6,070,454 to Cavestri; U.S. Pat. No. 6,070,455 to Cavestri; U.S. Pat. No. 6,101,867 to Cavestri; U.S. Pat. No. 6,150,306 to Friswell; U.S. Pat. No. 6,165,384 to Cooper et al.; U.S. Pat. No. 6,170,320 to Scaringe et al.; U.S. Pat. No. 6,786,960 to Profetto; and U.S. Pat. No. 6,840,990 to Gallagher et al., all of which are incorporated herein by reference.

### SUMMARY

Systems, methods, and compositions are described herein for treating transmission systems such that leaks may be detected and/or sealed. In some embodiments, the transmission system is a power transmission system. In some embodiments, the composition may include a carrier fluid, a transmission system sealant, and a light activated compound. The transmission system sealant may at least partially seal leaks in a transmission system during use. The light activated compound may be visible to the human eye when activated with an activating light. The light activated compound may fluoresce when treated with activating light.

Transmission systems may be treated with a composition by the methods described herein. A composition may be introduced into the transmission system. The composition may include a transmission system sealant and a light activated compound. After introduction of the composition, the transmission system may be operated for a period of time. Activating light may be directed towards at least a portion of the exterior of the transmission system to detect any light activated compound leaking from the power transmission system.

In some embodiments, activating light may be directed towards at least a portion of the exterior of the transmission system after inhibiting one or more leaks detected during a previous inspection of the transmission system.

In some embodiments, the composition may be provided as a kit. The kit may include an activating light source.

### DETAILED DESCRIPTION

Systems, methods, and compositions described herein relate to sealing and detecting of leaks in transmission systems. "Transmission system" refers to a manual transmission system, a power transmission system, or a continuously vari-

able system. Manual transmission systems include, but are not limited to, a gear selector fork, a collar, a layshaft, and gears. Power transmissions include, but are not limited to, gears, turbines, torque converters, gear pumps, lubricant lines, transmissions coolers, governors, valves, seals, lubricant addition ports, and solenoids. In some embodiments, gears of a transmission system may be referred to as planetary gears. Transmissions may be positioned in, but not limited to, machinery that includes gears that have the ability to be changed. Machinery includes, but is not limited to, motorized vehicles, bicycles, and drilling systems. Examples of motorized vehicles include, automobiles, trucks, buses, off-highway vehicles, refuse trucks, fire trucks, emergency vehicles, and electric drive vehicles. Examples of drilling systems include, but are not limited to, oil field drilling rigs and/or water drilling rigs.

A transmission system may exhibit leaks that may be observed by the human eye. For example, droplets of transmission lubricant may be observed on a surface of a component of the transmission system and/or on a surface beneath the transmission system (e.g., ground, asphalt surface, cement surface, tile surface, or combinations thereof). "Transmission lubricant" refers to a fluid that has a viscosity of at least 5 centistokes at 40° C. and/or a thixotropic substance. In some embodiments, transmission systems may exhibit leaks that may not be readily detected by the human eye. For example, transmission lubricant from leaks that develop when the transmission system is operated may disperse into the air without being detected. Leaks in a transmission system may result in diminished performance of a transmission system. Diminished performance of a transmission system may lessen the system's ability to transmit power, change gears, and/or may cause the gears to seize.

Leaks may be inhibited in transmission systems by replacement of seals, gaskets, or other transmission components. Replacement of transmission system components may be expensive and/or time consuming. The ability to inhibit or stop a leak without replacement of transmission components may allow a transmission system to be operated without loss of time ("downtime") due to repairing the transmission. Limited downtime may enhance productivity of commercial operations that rely on transmission systems for transportation and/or power.

In some embodiments, after the transmission system has been operated for a period of time and after repairing a leak in the transmission system, an area around the transmission system may be inspected (e.g., by looking for transmission system lubricant) to determine if the leak has ceased. Alternatively, a light activated compound may be added to the transmission system, circulated through the system, and detected using an activating light source. An activating light source includes, but is not limited to, sunlight and/or an ultraviolet (UV) light source. If no lubricant and/or dye visualization is observed, the leak is determined to be stopped.

Early detection of a different leak in the transmission system or of a leak from the same area in the transmission system may prevent lost time and/or expensive repairs. Typically, most dyes used for detection decompose and/or vaporize after the transmission is operated for a period of time. In certain embodiments, a light activated compound may be used that is not substantially decomposed and/or vaporized under typical transmission system operating conditions.

In some embodiments, a composition that includes a transmission system sealant and a light activated compound may be used to detect and seal one or more leaks in the transmission system. "Sealant" refers to a compound, a mixture of compounds, particles, or combinations thereof that inhibit

passage of liquid and/or gas from one area to a different area. The composition may include a carrier fluid, a transmission system sealant, and a light activated compound. In some embodiments, the transmission system sealant is a power transmission system sealant. The composition may also include additives such as pour point depressants, viscosity modifiers, friction modifiers, extreme pressure additives, dispersants, anti-foam agents, metal deactivators, surfactants, preservatives, corrosion inhibitors, antioxidants, fragrances, visible dyes, or mixtures thereof. In some embodiments, surfactants may enhance the miscibility of the composition with the transmission lubricant in the transmission system.

A carrier fluid may include fluids that are compatible with a transmission lubricant used in the transmission system. Examples of carrier fluids include, but are not limited to, hydrocarbons, refined petroleum compounds, alcohols, poly-alcohols (e.g., polyalkylene glycol (PAG)), esters, polyol esters, poly-alpha olefins (PAO), silicone fluids, or mixtures thereof.

Hydrocarbons include compounds that are composed of compounds that contain only hydrogen and carbon. In some embodiments, hydrocarbons include compounds having at least five carbon atoms. In some embodiments, hydrocarbons may have a carbon number from 5 to 50, from 10 to 40, or from 20 to 30. Hydrocarbons include, but are not limited to, alkyl compounds, olefins, aryl compounds, cyclic compounds, or mixtures thereof. Examples of hydrocarbons include, but are not limited to, hexane, toluene, substituted toluene, benzene, substituted benzenes, cycloparaffins, cyclohexanes, naphthalene, octanes, iso-octane, or mixtures thereof. In some embodiments, the composition may include from about 0.1 grams to about 99 grams, from about 1 gram to about 90 grams, from about 10 grams to about 80 grams, from about 20 grams to about 70 grams, from about 30 grams to about 60 grams, or from about 40 grams to about 50 grams of hydrocarbons per 100 grams of composition.

Refined petroleum compounds include compounds that have been produced from hydrocarbon sources (e.g., oil). In some embodiments, refined petroleum compounds may include hydrocarbons, compounds containing heteroatoms (e.g., sulfur, nitrogen, or phosphorus), compounds having a carbon number of at least 1, or mixtures thereof. In some embodiments, refined petroleum compounds include a mixture of cycloparaffins and aromatics (e.g., naphthenic oils). For example, refined petroleum compounds may include greater than 80 grams, greater than 90 grams, or greater than 99 grams of naphthenic oil per 100 grams of refined petroleum compounds. In some embodiments, the refined petroleum compounds may have a viscosity in a range from about 50 SUS to about 150 SUS, from about 75 SUS to about 125 SUS, or from about 90 SUS to about 110 SUS at 100° C.

Poly-alpha olefins include compounds having a molecular weight from about 600 to about 3,000,000 and result from the polymerization of one or more alpha-olefins. Examples of alpha-olefins that may be converted to poly-alpha olefins include, but are not limited to, ethylene, propylene, 1-butene, 1-pentene, 4-methyl-1-pentene, 1-hexene, or mixtures thereof. In some embodiments, the composition may include from about 0.01 grams to about 50 grams, from about 0.1 grams to about 30 grams, or from about 1 gram to about 20 grams of poly-alpha olefins per 100 grams of composition.

“Alcohols” refer to compounds having at least one hydroxy (OH) group. In some embodiments, alcohols include compounds having the general formula of  $C_nH_{2n+1}OH$ , where n is at least 1. Examples of alcohols include, but are not limited to, methanol, ethanol, propanol, iso-propanol, butanol, sec-butanol, tert-butanol, or mixtures thereof. In some embodi-

ments, alcohols may be combined with a carrier fluid to enhance solubility and/or dispersion of a transmission system sealant, a light activated compound, additives, or mixtures thereof combined in the carrier fluid.

“Esters” refer to compounds or mixtures of compounds having the general formula of  $RCO_2R'$  where R and R' are alkyl and/or aryl. Examples of esters include, but are not limited to, methyl acetate, ethyl acetate, stearin, palmitin, methyl butanoate, methyl salicylate, methyl benzoate, ethyl methanoate, ethyl butanoate, pentyl ethanoate, pentyl pentanoate, pentyl butanoate, octyl ethanoate, methyl stearate, esters of dicarboxylic acids, or mixtures thereof. Examples of esters of dicarboxylic acids include, but are not limited to, alkyl or aryl esters formed from: phthalic acid, succinic acid, alkyl succinic acids and alkenyl succinic acids, maleic acid, azelaic acid, suberic acid, sebacic acid, fumaric acid, adipic acid, linoleic acid dimer, malonic acid, alkyl malonic acids, alkenyl malonic acids, 1,2-benzenedicarboxylic acid diisonylon ester, or mixtures thereof. Esters may be combined with a carrier fluid to enhance solubility and/or dispersion of a transmission system sealant, a light activated compound, additives, or mixtures thereof that are combined with the carrier fluid. Esters may, in some embodiments, be used as a fragrance in the composition. In some embodiments, the composition may include from about 0.01 grams to about 50 grams, from about 0.1 grams to about 30 grams, or from about 1 gram to about 20 grams of ester per 100 grams of composition.

Polyol esters include, but are not limited to, glycerol esters, sorbitan esters, pentaerythritol esters, trimethylolpropane esters, or mixtures thereof. In some embodiments, the composition may include from about 0.01 grams to about 50 grams, from about 0.1 grams to about 30 grams, or from about 1 gram to about 20 grams of esters per 100 grams of composition.

In some embodiments, esters may include phosphate esters. Examples of phosphate esters include, but are not limited to, dialkyl phosphate esters, alkyl diaryl phosphate esters (e.g., 2-ethylhexyl diphenyl phosphate or isodecyl diphenyl phosphate), diaryl phosphate esters, triarylphosphate esters (e.g., tricresyl phosphate or isopropylated triphenyl phosphate ester), butylated triphenyl phosphate ester (e.g., tetra-butyl triphenyl phosphate), trimester alkyl phosphate esters (e.g., trisbutoxyethyl phosphate), or mixtures thereof. In some embodiments, esters containing a heteroatom may be used as extreme-pressure additives, anti-wear additives, plasticizers, or flame retardants. In some embodiments, the composition may include from about 0.01 grams to about 50 grams, from about 0.1 grams to about 30 grams, or from about 1 gram to about 20 grams of phosphate esters per 100 grams of composition.

“Alcohol ethers” refer to compounds or a mixture of compounds having the general formula of  $H(OCH_2CH_2)_nOR'$ , where R' is alkyl and/or aryl, and n is at least 1. Examples of alcohol ethers include, but are not limited to, cellulose ethers, grafted polyol ethers, and ethylene glycol ethers (e.g., glycol propyl ether, ethylene glycol monobutyl ether, or ethylene glycol monobenzyl ether). In some embodiments, alcohol ethers may be combined with a carrier fluid to enhance solubility and/or dispersion of a transmission system sealant, a light activated compound, additives, or mixtures thereof that are combined in the carrier fluid. In some embodiments, the composition may include from about 0.01 grams to about 50 grams, from about 0.1 grams to about 30 grams, or from about 1 gram to about 20 grams of alcohol ethers per 100 grams of composition.

Antioxidants include, but are not limited to, metal salts of dialkyl dithiophosphates, alkylated diphenyl amines, sulfurized alkylphenols and phenolates, hindered phenols, or mixtures thereof. Metals of metal salts of dialkyl dithiophosphates include, but are not limited to, metals from Columns 6-12 of the Periodic Table (e.g., zinc, cadmium, or molybdenum). "Periodic Table" refers to the Periodic Table as published by the International Union of Pure and Applied Chemistry on Nov. 7, 2003. In some embodiments, the composition may include from about 0.001 grams to about 10 grams, from about 0.01 grams to about 5 grams, or from about 0.1 grams to about 1 gram of antioxidant per 100 grams of composition.

Antifoamants include, but are not limited to, silicones, polysilicones, or mixtures thereof. In some embodiments, the composition may include from about 0.00001 grams to about 1 gram, from about 0.0001 grams to about 0.1 grams, or from about 0.001 grams to about 0.01 grams of antifoamant per 100 grams of composition.

Corrosion inhibitors include, but are not limited to, metal salts of dialkyl dithiophosphates, metal sulfonate salts, metal phenolate salts, or mixtures thereof. Metals of metal sulfonates and metal phenolates include, but are not limited to, metals from Columns 1 and 2 of the Periodic Table (e.g., calcium, barium, sodium, or magnesium). In some embodiments, the composition may include from about 0.0001 grams to about 10 grams, from about 0.001 grams to about 1.0 gram, or from about 0.01 grams to about 0.1 gram of corrosion inhibitor per 100 grams of composition.

Dispersants include, but are not limited to, polyisobutylene succinate esters, Mannich Base ashless dispersants, or mixtures thereof. In some embodiments, a polyisobutylene portion of a succinate ester may have a molecular weight ranging from about 500 to about 3,000 or from about 900 to from 2,500. In some embodiments, the composition may include from 0.5 grams to about 10.0 grams or from about 1 gram to about 3 grams of dispersant per 100 grams of composition.

Extreme-pressure additives include, but are not limited to, amine salts of phosphoric acids, dibenzyl polysulfides, di-tert-nonyl polysulfides, didodecyl polysulfides, di-tert-butyl polysulfides, dioctyl polysulfides, diphenyl polysulfides, dicyclohexyl polysulfides, zinc dithiophosphate, molybdenum sulfides, molybdenum organosulfides, or mixtures thereof. Extreme-pressure additives, in some embodiments, may perform as metal-deactivators, anti-wear additives, corrosion inhibitors, and/or friction modifiers. In some embodiments, the composition may include from about 0.01 grams to about 30 grams, from about 0.1 grams to about 20 grams, or from about 1 gram to about 10 grams of extreme-pressure additives per 100 grams of composition.

Friction modifiers may include, but are not limited to, alkane phosphonic acids, alkanols, amides, amines, alkanoamides, alkoxylated amines, alkoxylated ether amines, amine oxides, amidoamines, amino guanidines, amine salts, betaines, borated glycerol monooleates, glycerol esters of dimerized fatty acids, esters of carboxylic acids, esters of anhydrides, fatty acid esters, imidazolines, imines, nitriles, organo-molybdenum compounds, molybdenum dialkylthiocarbamates, molybdenum dialkyl dithiophosphates, molybdenum disulfide, tri-molybdenum cluster dialkylthiocarbamates, non-sulfur molybdenum compounds, quaternary amines, or mixtures thereof. Friction modifiers may, in some embodiments, perform as extreme-pressure additives, corrosion inhibitors, metal deactivators, and/or anti-wear additives. In some embodiments, the composition may include from about 0.01 grams to about 10 grams or from about 0.1 grams to about 1 gram of friction modifiers per 100 grams of composition.

Pour point depressants include, but are not limited to, polyacrylates, polymethacrylates, copolymers of ethylene and propylene, or polymers having a molecular weight from about 20,000 to about 120,000. In some embodiments, the composition may include from about 0.01 grams to about 10 grams or from about 0.1 gram to about 1 grams of pour point depressant per 100 grams of composition.

Viscosity modifiers include, but are not limited to, polyisobutylene, copolymers of ethylene and propylene and higher alpha-olefins, polymethacrylates, polyalkylmethacrylates, methacrylate copolymers, copolymers of an unsaturated dicarboxylic acid and a vinyl compound, inter polymers of styrene and acrylic esters, and partially hydrogenated copolymers of styrene/isoprene, styrene/butadiene, and isoprene/butadiene, as well as the partially hydrogenated homopolymers of butadiene and isoprene and isoprene/divinylbenzene. In some embodiments, the composition may include from about 0.01 grams to about 20 grams or from about 1 gram to about 10 grams of viscosity modifier per 100 grams of composition. In some embodiments, viscosity modifiers may function as a dispersant.

Surfactants include, but are not limited to, anionic surfactants, cationic surfactants, non-ionic surfactants, amphoteric surfactants, or mixtures thereof. In some embodiments, surfactants may enhance the miscibility of the composition with the fluid in the transmission system. Examples of anionic surfactants include, but are not limited to, phenates, salicylates, overbased sulfonates, neutral sulfonates, or linear alkyl benzene sulfonates. Examples of cationic surfactants include, but are not limited to, alkyl pyridinium compounds and/or quaternary ammonium compounds. Examples of amphoteric surfactants include, but are not limited to, imidazolines and betaines. Examples of nonionic surfactants include, but are not limited to, alkyl phenol ethoxylates, alkyl ethoxylates, alkylpolyglycosides, polyhydroxy long-chain carboxylic acid amides, long-chain carboxylic acid salts, sulfonates, phosphonates, sulfate and phosphate-based compounds capable of dissolving in water, or mixtures thereof. "Long-chain carboxylic acids" refer to saturated and unsaturated carboxylic acids having between 6 and 30 carbon atoms. In some embodiments, the composition may include from about 0.01 grams to about 30 grams, from about 0.1 grams to about 20 grams, or from about 1 gram to about 10 grams of surfactant per 100 grams of composition.

Carrier fluids and/or additives are commercially available from Asahi Denka Kogyo K. K. (Japan), Akzo Nobel Chemicals (Netherlands), Chevron Oronite (Houston, Tex., U.S.A.), Chemtura (Middlebury, Conn., U.S.A.), Degussa-RohMax USA (Horsham, Pa., U.S.A.), ExxonMobile Co. (Houston, Tex., U.S.A.), Infineum (United Kingdom), Lubrizol (Cleveland, Ohio, U.S.A.), R. T. Vanderbilt Company, Inc. (Norwalk, Conn.), Shell Chemical Co. (Houston, Tex., U.S.A.), or Shell Oil Co. (Houston, Tex., U.S.A.). In some embodiments, a mixture of a carrier fluid, one or more additives, and/or one or more light activated compounds may be commercially available as a formulated package.

"Light activated compounds" refer to a compound or compounds that are visible to the human eye when exposed to activating light (e.g. UV light or sunlight). Light activated compounds may include fluorescent dyes and/or phosphorescent dyes. Fluorescent dyes and/or phosphorescent dyes may have a visible color or may be colorless. Fluorescent dyes that may not be visible to a human eye may be visible when the fluorescent dye is treated with ultraviolet light. In some embodiments, a light activated compound may remain substantially unchanged when heated up to 1000° C., up to 800° C., up to 600° C., or up to 400° C. Light activated compounds

may be available as a solid or a liquid. In some embodiments, the composition may include from about 0.00001 grams to about 10 grams, from about 0.001 grams to about 1 gram, or from about 0.01 grams to about 0.1 gram of light activated compound per 100 grams of composition.

Light activated compounds include, but are not limited to, the following compounds or derivatives of the following compounds: anthracenes, aminoalkylphenothiazines, aminophenylbenzothiazoles, benzothiazolines, benzothiazoles, benzotriazoles, carbazoles, coumarins, diphenylamines, fluoresceins, naphthalenes, naphthalamides, naphthylamides, naphthylimides, phenanthracenes, phenothiazines, perylenes, pyrrolidones, phenols, quinolines, isoquinolines, purines, thioxanes, thioxanthanes, and 1,3,4-thiadiazoles. Examples of these compounds include, but are not limited to, coumarin 6; coumarin 7; coumarin 30; coumarin 6H; coumarin 102; coumarin 110; coumarin 152; coumarin 153; coumarin 314; coumarin 334; coumarin 337; coumarin 343; coumarin 480D; coumarin-3-carboxylic acid; 7-(2H-naphtho[1,2-D]triazol-2-yl)-3 phenylcoumarin; 2-aminobenzothiazole; benzothiazole; N-phenyl-1-naphthylamine; N-phenyl-2-naphthylamine; N-(4-cumylphenyl)-1-naphthylamine; p-tert-dodecylphenyl-2-naphthylamine; 2,2-dimethylbenzothiazoline; bis(benzothiazoline); benzotriazole; methylene bis(dibutyl dithiocarbamate); 2,6-di-tert-butyl-4-methylphenol; 2,5-dimercapto-1,3,4-thiadiazole; dioctyldiphenylamine; didecyldiphenylamine; or 1-methyl-2-pyrrolidone. Organic metallics such as molybdenum dialkylphosphorodithioate and zinc octyldithio-phosphate; and inorganic compounds such zinc sulfide and cadmium sulfide also may be used as light activated compounds.

Light activated compounds are commercially available as STAY BRITE® BSL 712, STAY BRITE® BSL 713, STAY BRITE® BSL 714 (Brite Solutions, Troy Mich., U.S.A.), DAY GLOW® TRY-33 (Day Glow Color Corp, Cleveland, Ohio, U.S.A.), R-12 dye (part 16252, SPX Corporation, Robinair, Montpelier, Ohio, U.S.A.), or R-134a dye (part 16253, SPX Corporation, Robinair, Montpelier, Ohio, U.S.A.), D15000 (Chromatech, Inc., Canton, Mich., U.S.A.), Solvent Yellow 43 (Keystone Aniline Corporation, Chicago, Ill., U.S.A.). Other sources for light activated compounds are Aldrich Chemical Co. (Milwaukee, Wis., U.S.A.) and Rohm and Haas (Philadelphia, Pa., U.S.A.).

The composition may include a transmission system sealant capable of stopping and/or inhibiting the leak. The transmission system sealant may include material such as polymeric material, plasticizers, synthetic fibers, cellulose fibers, or combinations thereof. Polymeric material include, but are not limited to, latex, polyvinyl acetate, polyvinyl resins, or mixtures thereof.

Plasticizers include, but are not limited to, phthalate esters, aliphatic dibasic acid esters, trimellitates, pyromellitic acid esters, phosphates, and/or refined hydrocarbons. In some embodiments, a mixture of aromatic hydrocarbons, diisononyl phthalate, and dialkyl phosphate esters may perform as a sealant for the engine system. Examples of phthalate esters such as di(2-ethylhexyl) phthalate, butyl benzyl phthalate, dinonyl phthalate, diisononyl phthalate, diisodecyl phthalate, diundecyl phthalate, diheptyl phthalate, butyl phthalyl, butyl glycolate. Examples of aliphatic dibasic acid esters include diethyl adipate, didecyl adipate, diethyl sebacate; polyglycol benzoates such as polyoxyethylene glycol dibenzoate, polyoxypropylene glycol dibenzoate.

In some embodiments, the composition may include from about 1 gram to about 99 grams, from about 10 grams to about 90 grams, from about 20 grams to about 80 grams, from about

30 grams to about 70 grams, or from about 40 grams to about 60 grams of sealant per 100 grams of composition.

The transmission system sealant may be dispersed or emulsified in the carrier fluid. In some embodiments, the transmission system sealant may swell when heated in the transmission system. A swellable material may allow transmission system sealant of relatively small diameter to be introduced into the transmission system and not be removed by filters positioned in the transmission system. The transmission system sealant may enlarge (swell) as the composition is circulated through the transmission system.

In some embodiments, visible light activated dyes (e.g., visible dyes such as green, blue or red dyes) may be added to the composition. In some embodiments, dyes may be used to differentiate the composition from other leak detecting and/or leak sealing products. A composition may include up to 1 grams, up to 0.5 grams, or up to 0.01 grams of dye, per 100 grams of composition.

A composition may be formed by mixing a carrier fluid, one or more light activated compounds, and one or more transmission system sealant. In some embodiments, a carrier fluid, one or more additives, one or more light activated compounds, and one or more transmission system sealants may be mixed together. Mixing of the ingredients may be performed at a temperature ranging from about 10° C. to about 200° C., from about 25° C. to about 100° C., or from about 50° C. to about 90° C. The combined ingredients may be mixed for about 0.5 hour, about 1 hour, about 2 hour, or up to 24 hours to form the composition. In some embodiments, the transmission system sealant may be partially soluble and/or suspended in the composition. Table 1 lists representative ranges of compounds in compositions to detect and seal leaks in a transmission system.

TABLE 1

| Compound                       | Volume % (based on total volume of composition) |    |    |    |    |    |    |    |    |    |
|--------------------------------|-------------------------------------------------|----|----|----|----|----|----|----|----|----|
|                                | 1                                               | 2  | 3  | 4  | 5  | 6  | 7  | 8  | 9  | 10 |
| 40 Refined Petroleum Compounds | 27                                              | 21 | 39 | 43 | 47 | 53 | 57 | 62 | 64 | 65 |
| Anti-foamant                   | —                                               | —  | <1 | —  | <1 | —  | <1 | —  | —  | —  |
| Dispersant                     | 5                                               | —  | 5  | 5  | 5  | —  | —  | —  | —  | —  |
| Friction modifier              | —                                               | —  | —  | —  | 1  | —  | —  | —  | —  | —  |
| Ester                          | —                                               | 20 | 15 | —  | 10 | —  | 15 | 10 | —  | —  |
| Phosphate ester                | —                                               | 5  | 10 | —  | 10 | 20 | —  | 10 | 15 | —  |
| Alcohol ether                  | 20                                              | 30 | 21 | 10 | 10 | 15 | 8  | 5  | 5  | 3  |
| Pour Point Depressant          | —                                               | 1  | —  | —  | —  | —  | 2  | —  | —  | —  |
| Sealant                        | 40                                              | 20 | 5  | 35 | 10 | 10 | 15 | 10 | 15 | 30 |
| Surfactant                     | 5                                               | —  | —  | 5  | 5  | —  | —  | —  | —  | —  |
| UV dye                         | 3                                               | 3  | 1  | 2  | 1  | 2  | 2  | 3  | 1  | 2  |
| 50 Viscosity modifier          | —                                               | —  | 2  | —  | —  | —  | —  | —  | —  | —  |

55 In some embodiments, the composition may be packaged in a clear bottle, colored bottle, or metal can. The bottle may be composed of polymeric material and/or glass. The bottle and/or can may include an end that is tapered. A tapered end may allow the composition to be added directly to a port of the transmission system. In some embodiments, the composition may be added to a transmission lubricant port of the transmission system using a funnel, a hand pump, or other pressurized pumping system.

60 In some embodiments, a composition may be sold and/or packaged as part of a kit. The kit may include safety glasses, towels, funnels, an activating light source such as an UV light, or combinations thereof. The kit may be packaged in a carrying case with pre-formed segments to hold the components of the kit. In some embodiments, the carrying case may be

plastic and/or include a handle. In some embodiments, the pre-formed segments may be removable.

In some embodiments, a transmission system may be treated with a composition as described herein to detect and/or seal leaks in the transmission system. In certain embodiments, the transmission system is a power transmission system. In other embodiments, the transmission system is a manual transmission system. The composition may be added directly to a transmission system through the transmission lubricant port. In some embodiments, the transmission system may be treated with the composition at the site of manufacture. Addition of the composition at the site of manufacture may enable leaks that develop during the manufacturing process and/or during shipment of new machinery to be detected and sealed.

In some embodiments, the composition may be pre-mixed with transmission lubricant to form a transmission lubricant/composition mixture. Once mixed, the transmission lubricant/composition mixture may be added to a transmission system through the transmission lubricant port.

Once added to the transmission system, the composition is circulated through the transmission system for a period of time. For example, the composition may be circulated by operating the transmission system for at least 1 minute, at least 60 minutes, at least 4 hours, at least 8 hours, at least 3 days, at least 4 days, or up to about 1 week. After circulating the composition through the transmission system, activating light (e.g. UV light) may be directed towards at least a portion (e.g. the exterior of) one or more components of the transmission system. If a leak is present in the transmission system, the light activated compound would be visible to the eye when activated by the activating light.

Visualization of the light activated compound(s) under an activating light source may indicate the source(s) of the leak(s). Once the source(s) of the leak(s) are detected, the composition may be removed from the site of the source. For example, a person may wipe a cloth over a seal to remove any transmission lubricant from the seal. The composition may then be continuously circulated through the transmission system for a period of time. As the composition circulates through the transmission system, the leak may be sealed with the transmission system sealant. The leak area may be monitored with the activating light source. Confirmation that the leak is sealed may be obtained by directing activating light towards the exterior of the transmission system and noting when little or none of the light activated compound is detected.

In some embodiments, the transmission system may be monitored for leaks over a period of time. For example, after a period of time and/or a number of miles, activating light may be directed towards a portion of the transmission system to determine if the previously sealed leak is still sealed, or if any new leaks are present. Examples of time periods include, but are not limited to, at least 50 hours, at least 100 hours, at least 500 hours, at least 700 hours, at least 1,000 hours, at least 1,500 hours, at least 2,000 hours, or at least 30,000 hours. Examples of miles include, but are not limited to at least 1,000 miles, at least 2,000 miles, at least 3,000 miles, at least 5,000 miles, or at least 7,500 miles. In some embodiments, the composition may be removed from the transmission system by removing the transmission lubricant from the system and/or flushing the transmission system with fresh transmission lubricant.

In this patent, certain U.S. patents have been incorporated by reference. The text of such U.S. patents is, however, only incorporated by reference to the extent that no conflict exists between such text and the other statements and drawings set forth herein. In the event of such conflict, then any such

conflicting text in such incorporated by reference U.S. patents is specifically not incorporated by reference in this patent.

Further modifications and alternative embodiments of various aspects of the invention may be apparent to those skilled in the art in view of this description. Accordingly, this description is to be construed as illustrative only and is for the purpose of teaching those skilled in the art the general manner of carrying out the invention. It is to be understood that the forms of the invention shown and described herein are to be taken as the presently preferred embodiments. Elements and materials may be substituted for those described herein, processes may be reversed, and certain features of the invention may be utilized independently, all as would be apparent to one skilled in the art after having the benefit of this description to the invention. Changes may be made in the elements described herein without departing from the spirit and scope of the invention as described in the following claims. In addition, it is to be understood that features described herein independently may, in certain embodiments, be combined.

What is claimed is:

1. A method for treating a transmission system, comprising:
  - introducing a composition into the transmission system, the composition comprising one or more transmission system sealants, one or more fluids compatible with a transmission system lubricant of the transmission system, and one or more light activated compounds, wherein the transmission system sealant(s) inhibit one or more leaks of the transmission system during use;
  - operating the transmission system after introducing the composition into the transmission system; and
  - directing activating light towards at least a portion of the transmission system, wherein one or more of the light activated compounds are visible when treated with the activating light during use.
2. The method of claim 1, further comprising directing activating light toward at least a portion of the transmission system after inhibiting one or more leaks detected during a previous inspection of the transmission system.
3. The method of claim 1, wherein the activating light is ultraviolet light.
4. The method of claim 1, wherein at least one of the light activated compounds comprises a fluorescent compound.
5. The method of claim 1, wherein at least one of the light activated compounds comprises a perylene.
6. The method of claim 1, wherein one or more of the light activated compounds remain substantially unchanged at temperatures of up to about 1000° C.
7. The method of claim 1, wherein the one or more transmission system sealants comprise one or more phosphate esters.
8. The method of claim 1, wherein the one or more transmission system sealants comprise one or more alkyl phthalates.
9. The method of claim 1, wherein the one or more transmission system sealants comprise synthetic fibers.
10. The method of claim 1, wherein the one or more transmission system sealants comprise one or more esters.
11. The method of claim 1, wherein the one or more transmission system sealants comprise one or more triarylphosphate esters.
12. The method of claim 1, wherein the composition further comprises refined petroleum compounds.
13. The method of claim 1, wherein the composition further comprises a surfactant.